

# UNITED STATES PATENT OFFICE.

HENRY HESS, OF PHILADELPHIA, PENNSYLVANIA.

## METHOD OF COATING ARTICLES.

1,252,005.

Specification of Letters Patent.

Patented Jan. 1, 1918.

No Drawing.

Application filed June 23, 1916. Serial No. 105,402.

To all whom it may concern:

Be it known that I, HENRY HESS, a citizen of the United States, residing at Philadelphia, in the county of Philadelphia and 5 State of Pennsylvania, have invented certain new and useful Improvements in Methods of Coating Articles, of which the following is a specification.

This invention relates to the coating of 10 metal articles, the object of the invention being to apply a metal coating to small miscellaneous metal articles such as screws, nails and small hardware of iron, steel and other metals, in such manner that the coating will 15 be applied smoothly and uniformly and large numbers of the articles may be treated expeditiously and economically.

In accordance with my invention I employ 20 a coating composition containing a metal ingredient which is capable of fusion with the metal of the article to be coated, and I first cover the articles with this composition and then subject the coated articles to heat sufficient to melt the metal ingredient, whereby 25 it will fuse with the metal of the articles and completely coat the same.

Various coating compositions which will 30 act in this manner under the conditions mentioned are known, the metal ingredient in some cases being tin to apply a tin coating and in other cases lead to apply a lead coating and other metals in still other cases according to the character of the coating to be applied.

35 A suitable composition where a tin coating for instance is to be applied may consist of two kilo. tin powder, one kilo. of powdered chlorid of zinc to act as a deoxidizing and fluxing agent and a neutral liquid to dissolve the fluxing substance, for instance water or 40 alcohol. For applying a lead coating the same ingredients may be employed except that powdered lead will be substituted for powdered tin.

45 I propose, in accordance with my invention, to handle the articles to be coated *en masse* or in bulk, for instance by placing a large number of the same in a suitable container, preferably a reticulated basket or 50 holder. The basket with the contained articles is then immersed in a liquid bath of the coating composition, and allowed to remain a sufficient time to permit the composition to reach all portions of the mass and 55 completely cover the individual articles.

The complete covering of the articles by the

composition may be aided and facilitated by stirring the composition or agitating the container in the bath. When the articles have become thoroughly covered with the composition the container is lifted out and the surplus material allowed to drain off, or the container may be agitated or subjected to a rotary motion to expel the surplus material by centrifugal force. The articles with the 60 composition thus applied are now subjected to heat of a degree sufficient to melt the metal ingredient of the composition in order to cause it to fuse or amalgamate with the surface metal of the articles and coat 65 the same. The articles may be subjected to heat in any suitable and appropriate manner, for instance by transferring the container with the articles therein to a suitable oven capable of producing sufficient heat 70 for the purpose mentioned. After the heat treatment the articles are removed from the oven and may then be subjected to a further manipulation in order to more completely remove any of the composition which might 75 adhere, and finally the coated articles are subjected, preferably while hot, to a tumbling action in order to prevent them from sticking to each other and to more thoroughly and uniformly distribute the coating and smooth down and polish the same. This tumbling action may be effected by 80 transferring the articles to a tumbling barrel or whizzer wherein the articles will be tumbled about against each other and by 85 their repeated impact with and attrition on each other, the coating will be evenly and uniformly distributed and will be smoothed down and the articles given a finished 90 polish.

95 Instead of placing the basket containing the cold covered articles in an oven to apply the fusing heat, the articles may be transferred from the basket to a tumbling barrel and the heat applied to the barrel 100 while the articles are being subjected therein to a tumbling action, the result of which operation will be to cause the fusion of the metal ingredient of the composition, and its amalgamation with the surface metal of 105 the articles, while at the same time the surplus composition is thrown off and the coating smoothed down and the articles polished by the attrition of the individual articles upon each other.

110 By my improved method of applying the metal coating, various kinds of small arti-

cles may be handled in large masses or collections and expeditiously and uniformly coated with a metal skin coating. The method of procedure is of peculiar advantage in the coating of barbed wire which may be handled in rolls or bales, with the barbs and sections of connecting wire constituting in effect a mass or collection of individual articles, in the handling of which 5 in the application of the coating, all portions of the barbs and connecting wire sections will be thoroughly covered and completely coated. The surplus coating composition may be removed from the barbed 10 wire bale by subjecting the latter to rapid rotation or whizzing action either before the heat application or subsequent thereto 15 or at both periods.

While I have described a coating composition consisting of tin or lead powder, 20 chlorid of zinc or chlorid of ammonium and water or alcohol as being suitable for carrying my improved method into effect, it will be understood that compositions containing 25 other ingredients may be employed provided that such compositions will contain a metal capable under the influence of heat of fusing or amalgamating with the surface metal of the article to be coated; and it will 30 be further understood that my method is not limited to any particular manner of procedure or sequence of steps except in so far as such limitations are specified in the claims.

35 Having thus described my invention, what I claim is:

1. The method of coating articles, which 40 consists in covering the articles *en masse* with a liquid coating composition containing an unmolten metal capable of fusion with the metal of the articles, manipulating the mass of articles to remove the surplus composition, and subjecting the covered articles *en masse* to heat sufficient to cause the 45 metal of the composition to fuse with the metal of the articles.

2. The method of coating articles, which 50 consists in covering the articles *en masse* with a liquid coating composition containing an unmolten metal capable of fusion

with the metal of the articles, manipulating the mass to remove the surplus composition, subjecting the covered articles *en masse* to heat sufficient to cause the metal of the composition to fuse with the metal of 55 the articles *en masse*, and further manipulating the coated articles while hot to free the same of surplus coating material.

3. The method of coating articles, which 60 consists in arranging said articles *en masse* in a suitable container, immersing the container in a liquid bath of coating composition containing an unmolten metal capable of fusion with the metal of the articles, removing the container from the bath and 65 manipulating the same to remove the surplus composition, and finally subjecting the mass of articles while in the container to heat sufficient to melt the metal of the composition and cause it to fuse with the metal 70 of the articles.

4. The method of coating articles, which 75 consists in covering the articles *en masse* with a liquid coating composition containing an unmolten metal capable of fusion with the metal of the articles, subjecting the covered articles *en masse* to heat sufficient to melt the metal and cause it to fuse with the metal of the articles, and subjecting the 80 coated articles while still hot to a tumbling action to smooth down the coating.

5. The method of coating articles, which 85 consists in arranging said articles *en masse* in a suitable container, immersing the container in a liquid bath of a composition containing an unmolten metal capable of fusion with the metal of the articles, removing the container and articles from the bath, manipulating the container and articles to throw off the surplus coating composition, 90 subjecting the coated articles *en masse* to heat sufficient to melt the metal of the composition and cause it to fuse with the metal of the articles, and removing the coated articles from the container and subjecting the 95 same to a tumbling action to smooth down the coating.

In testimony whereof, I have affixed my signature.

HENRY HESS.